

## UNITED STATES PATENT OFFICE

2,459,831

## PROCESS FOR DYEING NYLON WITH ACID DYES OF LIMITED SOLUBILITY

Frank C. McGrew and William Henry Sharkey,  
Wilmington, Del., assignors to E. I. du Pont de Nemours & Company, Wilmington, Del., a corporation of DelawareNo Drawing. Application July 2, 1946,  
Serial No. 681,136

6 Claims. (Cl. 8—55)

**1**  
This invention relates to the dyeing of textile fabrics, and more particularly to dyeing nylon fibers and fabrics.

In present commercial practice nylon is colored with a class of dyestuffs known as acetate dyes. These colors, although not highly sensitive to normal variations found in nylon yarn, are fugitive to washing. On the other hand, the classes of colors containing acid groups, e. g., carboxylic or sulfonic groups are known as acid or direct dyes and are characterized by good fastness to washing but show large differences in dye take-up from one part of the fiber to another. Yarns from different bobbins, i. e., spun at different times or from different lots of polymer, show this effect most clearly. In many cases, yarns from different bobbins, are colored to a different extent with acid dyes when dyed by standard dyeing procedures. As a result, nylon cloth dyed with these acid dyes is often colored in an uneven fashion, showing streaks and shade depth variations in knitted goods, and barré effects, warp streaks and the like in woven goods. This nonuniformity in dye behavior in the yarn is believed due to slight variations in chemical composition which cannot be completely controlled by present manufacturing processes, to variation in orientation (draw ratio) arising either in the spinning and processing of the yarn or in the mechanical action of the textile machinery used in the knitting or weaving of the yarn into fabrics, and perhaps to other, as yet unrecognized, causes.

This invention has as an object a new and improved process for dyeing nylon textile articles. A further object is a process for applying acid dyes uniformly on nylon yarn with evenness of color application and without the resulting streaks and shade depth variations that have previously characterized the acid dyeing of nylon fabrics. Other objects will appear hereinafter.

The above objects are accomplished by the method described below wherein the concentration of the dye is maintained highly dilute by means of an aqueous dyebath in which the dye is the salt of an acid dyestuff having but slight solubility in water.

We have discovered that the nylon fabrics, although subject to the difficulties in dyeing noted above with dyeing processes which are applicable to other fabrics and which require readily soluble dyestuff salts and their use in high concentration, are uniformly colored by conducting the dyeing in an aqueous dyebath in which the dyestuff salt is one which dissociates in the aqueous dyebath to yield a dye anion concentration of at least 0.1

**2**  
part per million but not greater than 50 parts per million based on the weight of the dyebath.

In one preferred method for carrying out this invention the desired amount of acid dyestuff is added to an aqueous bath containing an amount of barium chloride equal to 100—1000% of the weight of the nylon to be dyed and the mixture is stirred. The nylon fabric is added and the bath heated to 50—100° C. for a period of one hour. The nylon is removed from the dyebath, rinsed, and dried. Dyestuff is applied evenly on the nylon by this method even though draw ratio of the yarn used in preparation of the fabrics differs by as much as 4%. Similarly, even coloration is realized on fabrics prepared from yarns spun from different lots of nylon which, under normal dyeing conditions, show wide variations in depth of shade.

To accomplish the same result by an alternative method the barium salt of the dyestuff is first prepared, and then the nylon to be dyed is added. After heating until the dyestuff is taken up by the nylon, the fabric is removed from the bath.

The salts of the dyestuff used in the practice of this invention are of such low solubility that their use in excess, which is the preferred practice, of the amount required to yield the dye anion concentration within that previously stated will not increase this concentration beyond 50 parts per million based on the weight of the dyebath. In the alternative method mentioned above the aqueous bath to which the barium salt of the dyestuff is added can contain from 0% to 1000% barium chloride based on the fabric weight.

The synthetic linear polyamides known as nylon and the production of fibers and fabrics therefrom have been described in a number of United States patents and in particular in 2,071,250, 2,071,253 and 2,130,948. These fiber-forming polycarbonamides described in the previously mentioned patents are obtained by several methods, for example, by self-polymerization of a monoaminomonocarboxylic acid, e. g., 6-amino-caproic acid or 12-aminostearic acid, by reacting in substantially equimolecular proportions a di-basic acid, e. g., adipic or sebacic acid with a diamine, e. g., hexamethylenediamine or with a monoaminomonohydric alcohol, e. g., monoethanolamine, it being understood that these reactants can be replaced by their equivalent amide-forming derivatives. These linear polyamides also include polyesteramides, for example, those obtained by admixture with other linear polymer-forming reactants, such as glycol-dibasic acid mixtures, or mixtures of hydroxy acids, with

the previously mentioned polyamide-forming reactants. On hydrolysis with hydrochloric acid the amino acid polymers yield the amino acid hydrochloride, the diamine-dibasic acid polymers yield the diamine hydrochloride and the dibasic carboxylic acid, and the amino alcohol-dibasic acid polymers yield the amino alcohol hydrochloride and the dibasic carboxylic acid. In these polyamides the average number of carbon atoms separating the amide groups is at least 2. The preferred polyamides have an intrinsic viscosity of at least 0.4 (defined as in Patent 2,130,948) and a unit length (defined in Patents 2,071,253 and 2,130,948) of at least 7.

The following examples are further illustrative of the practice of this invention. Parts are by weight unless otherwise stated.

#### Example I

A dyebath is prepared by addition of 50 parts of water of 0.014 part of 1-benzoylamino-2-methyl-4- $\beta'$ -naphthylamino anthraquinone carbazole, 0.0025 part of milling yellow 5G, conc. (color index No. 642), and 0.0025 part of alizarin blue black B (color index No. 1085). To this is added 50 parts of a 5% calcium chloride solution (2.5 parts of  $\text{CaCl}_2$ ) and 0.1 part of acetic acid. The calcium salts of the dye separate leaving a colorless supernatant solution. This is stirred manually to disperse the color throughout the bath. To the bath is introduced 2 parts of a section of knitted nylon fabric prepared from yarns drawn respectively 3.82 and 3.99 (a difference of 4%) times its length as spun from the molten polymer. The bath is heated to 80° C. and held there for one hour as the fabric is manually agitated. The fabric is removed, rinsed, and dried. Inspection of the dyed fabric show it to be uniformly colored and devoid of spots or streaks and having no change in shade depth at the point where the yarns of different draw ratio were spliced together.

A similar section of nylon fabric knitted from the same yarns is dyed 1 hour at 80° C. with 0.014 part of 1-benzoyl-amino-2-methyl-4- $\beta'$ -naphthylamino anthraquinone carbazole, 0.0025 part of milling yellow 5G, conc. (color index No. 642) and 0.0025 part of alizarin blue black B (color index No. 1085) in an aqueous bath (100 parts) containing 0.1 part of acetic acid. The resulting dyed section shows a marked increase in shade depth at the point where the yarn of draw ratio 3.99 was spliced to the yarn of draw ratio 3.82 during knitting. Neither of the dyed pieces shows a visually perceptible change when tested for washing fastness according to Test Method 1 on page 187 of the 1940 Year Book of the American Association of Textile Chemists and Colorists, Vol. XVII.

#### Example II

A dyeing is conducted in the same manner as described in Example I except the barium chloride is substituted for the calcium chloride. The resulting fabric is uniformly colored and shows complete absence of spots, streaks, and shade depth variations.

#### Example III

A dyebath is prepared with the same dyes as given in Example I and in the same proportions. To this bath is added 10 parts of barium chloride and 0.04 part of acetic acid. The nylon fabric to be dyed is knit from two yarns spun at different times, both of which are drawn 3.55 times original length and both are processed alike. The

yarns are chosen so that the knit fabric shows a change in shade depth four times as great as that which is just perceptible to the eye at the point where they are spliced together when dyed by the conventional method as described in the latter part of Example I. Two parts of this knit fabric are added to the bath and the bath is heated to 80-85° C. for one hour and during this time the fabric is manually agitated. The nylon fabric is removed from the bath, rinsed, and dried. Examination of the piece shows that it is evenly colored and contains no light-shaded areas or spots.

#### Example IV

A dyebath is prepared by addition to 100 parts of water containing 10 parts of barium chloride of 0.0024 part of the product obtained by diazotization of 4-nitro-4'-aminodiphenylamine-2-sulfonic acid and coupling with o-cresol followed by condensation with p-toluene sulfonyl chloride, 0.0044 part of the product obtained by diazotization of 4-nitro-4'-aminodiphenylamine-2-sulfonic acid coupled to 1-aminonaphthalene-7-sulfonic acid and diazotizing and coupling to phenol and subsequently condensing with p-toluene sulfonyl chloride, and 0.0007 part of the product obtained by coupling diazotized 4-amino-4'-methylidiphenylamine-2-sulfonic acid to  $\alpha$ -naphthylamine followed by diazotization and coupling to 2-naphthol-6-sulfonic acid. A section of knit nylon fabric similar to that described in Example III and weighing two parts is introduced into this dyebath. The bath is heated to 80° C. in 15 minutes and maintained at 80-85° C. for one hour. Practically all of the color in the bath is taken up by the nylon. The nylon is removed from the bath, rinsed, and dried. It is uniformly colored, i. e., completely devoid of spots, streaks and shade depth variations. Dyeing a similar piece of fabric by conventional methods using the same dyes leads to a section of fabric that is much more deeply colored on one side than on the other.

In the practice of this invention the most important factor is the solubility of the salt of the dyestuff employed. Also important are the properties of the dyestuff itself, the cation employed, and the dyeing conditions under which the scantly soluble salt is used. These factors are all interdependent as will be explained.

It is preferred to employ salts of acid colors which dissociate in water to the extent of supplying 0.1 to 50 parts per million based on the dyebath of dye anion. This corresponds to a dye anion concentration no greater than  $10^{-5}$  moles per liter. Therefore, salts with a solubility product constant of at least  $10^{-14}$  and not greater than  $10^{-10}$  usually give better dyeings. However, satisfactory dyeings are obtained with salts having solubility product constants as high as  $10^{-5}$ , particularly if an excess of the precipitating cation is used at the same time to further reduce the concentration of the dye anion by the principle of mass action.

It has been found most convenient to use calcium or barium ions to form slightly soluble salts of acid and direct dyestuffs for use in dyeing as described in this invention. These cations are perfectly satisfactory for the great majority of acid and direct colors. However, other cations also form salts of low solubility with acid and direct dyestuffs, for example various alkaline earth metals such as strontium, and aliphatic, cycloaliphatic or aromatic ammonium ions containing at least five carbon atoms such as amyl-

ammonium, hexylammonium, cyclohexylammonium, dicyclohexylammonium, di(p-ammonium cyclohexyl) - methane, phenylammonium etc. ions. Certain other metallic ions such as ions of lead, aluminum, and magnesium form dye salts which meet the solubility requirements just recited. Some of these salts are less soluble than others and since such a wide range of precipitating cations is available, satisfactory combinations for all acid and direct dyestuffs can be obtained that will come within the solubility limits described above.

The character of the dyestuff has an important bearing also. For example, monobasic dyestuffs, i. e., containing one sulfonic acid group, form less soluble salts with alkaline earth metals and organic bases than do polybasic dyestuffs. However, these polybasic dyestuffs can be utilized in the practice of this invention although in some cases it is desirable to use the mass action principle to reduce solubility as described earlier. Satisfactory coverage of variations in yarn dyeing properties are ordinarily obtained with calcium or barium salts of practically all acid and direct dyes using as much as 100 to 1000% calcium chloride or barium chloride based on the weight of the nylon in the dyebath. In some cases where the calcium or barium salts do not meet the solubility limits given above, salts of di(p-ammonium cyclohexyl)methane, which meet solubility requirements with all but a very few acid and direct colors, are employed.

Dyeing conditions under which these scantily soluble salts of acid dyestuffs can be used vary quite widely. For example, they may be employed in baths in the pH range of 2-7 and at temperatures of 50-100° C. Temperatures greater than 100° C. may be used if the dyeing is done in pressure equipment. At low pH values, i. e., in the neighborhood of 2-4.5 it is not necessary to use excess barium chloride in the dyebath to suppress ionization of the salt with most colors whereas at higher pH values, i. e., 4.5-7, a substantial excess of the cation is necessary to result in uniform application of dye despite variations in the yarn. Temperature variations are not critical as any temperature from 20° C. to 100° C. can be used but for convenience it is preferred to keep within the range of 50-100° C. so that dyeing will be complete in 1 to 2 hours or less.

To obtain best uniformity with a minimum of agitation during dyeing it is desired to have the slightly soluble dye salt in a very fine state of subdivision so that a stable dispersion of the pigment may be prepared. Under such conditions the particles will perfuse the fabric completely and not be subject to any filtering action on the part of the fabric. To assist in preparation of stable dispersions of dye salts, dispersing agents may be used. This may be done by addition of the dispersing agent to the solution of dye before the precipitating cation is introduced to form the dye salt of low solubility or by treatment of the dye salt in a ball mill with an aqueous solution of the dispersing agent. Either non-ionic, cationic or anionic type dispersing agents may be used as illustrated respectively by polyvinylalcohol, dodecyl trimethylammonium bromide, and partially neutralized polymethacrylic acid.

The amount of dyestuff that may be applied by 70

the method of this invention is limited to substantially the same quantities that may be applied by conventional methods. That is, the use of dye salts of low solubility neither increases nor decreases the ability of nylon to absorb dyestuff but constitutes a process for applying uniformly on nylon the same amounts of color as can be applied by usual methods.

10 The apparatus used in the practice of this invention is of conventional type and should be designed to agitate the fabric and have arrangements for applying heat. Any of the various machines now in use for textile coloration are satisfactory.

15 It will be seen from the foregoing description that this invention provides a practical and economical method for effecting uniform application of washfast acid and direct dyestuffs on nylon yarns and fabrics even though wide variations in amount of dye take-up are encountered when dyed by conventional methods, regardless of the causes of these variations.

20 As many widely different embodiments of this invention may be made without departing from 25 the spirit and scope thereof, it is to be understood that this invention is not to be limited to specific embodiments thereof, except as defined in the appended claims.

We claim:

- 30 1. A process for evenly dyeing nylon textile articles which comprises immersing the nylon article, until the desired depth in shade is obtained, in an aqueous dyebath in which the coloring material is a salt of an acid dyestuff which 35 dissociates in the aqueous dyebath to yield a dye anion concentration of at least 0.1 part per million but not greater than 50 parts per million based on the weight of the dyebath.
2. The process set forth in claim 1 in which 40 the coloring material is an alkaline earth metal salt of an acid dyestuff.
3. The process set forth in claim 1 in which 45 said salt is a salt of the acid dyestuff with a multivalent metal ion.
4. The process set forth in claim 1 in which 50 said salt is the barium salt of the acid dyestuff.
5. The process set forth in claim 1 in which said salt is the calcium salt of the acid dyestuff.
6. The process set forth in claim 1 in which 55 said salt is the lead salt of the acid dyestuff.

FRANK C. McGREW.  
WILLIAM HENRY SHARKEY.

#### REFERENCES CITED

The following references are of record in the file of this patent:

#### UNITED STATES PATENTS

60 Number Name Date  
1,873,628 Ohlendorf \_\_\_\_\_ Aug. 23, 1932

#### FOREIGN PATENTS

Number Country Date  
65 22,097 Great Britain \_\_\_\_\_ 1908  
429,475 France \_\_\_\_\_ July 19, 1911

#### OTHER REFERENCES

Badische (Fr.) Addition 12,403 (2nd addition to basic Patent 297,330) June 20, 1910.